

Dec. 20, 1932.

L. J. O'MALLEY

1,891,776

SELECTIVE SEPARATION OF ORES

Filed June 14, 1930

*Fig. 1.*



*Fig. 2.*



*Fig. 3.*



*Inventor:*

*Louis J. O'Malley*

*By Emery Barth Barnes & Townsend Attorneys*

## UNITED STATES PATENT OFFICE

LOUIS J. O'MALLEY, OF BOSTON, MASSACHUSETTS

## SELECTIVE SEPARATION OF ORES

Application filed June 14, 1930. Serial No. 461,093.

My invention relates to methods of and apparatus for separating ores by froth flotation.

The invention will be best understood from the following description of an example of the practice of the method and from the accompanying drawing of one embodiment of apparatus for use in the practice of said method.

10 In the drawing:—

Fig. 1 is a longitudinal section of a Fahrenwald type flotation machine having applied thereto a pair of electrodes for improving the separation of the ore in accordance with

15 the invention;

Fig. 2 is a section on the line 2—2 of Fig. 1; and

Fig. 3 is a diagram illustrating schematically a bubble with an adhering ore particle.

Referring to the drawing, the flotation machine illustrated comprises a container 1 for the ore pulp and frothing liquid, the container having a submerged partition 3 which provides an auxiliary chamber 5. At the lower end of the chamber 5 is a pump impeller 7 separated from the body of said chamber by a hood and baffle arrangement 9. The impeller 7, as shown, is rotated by a shaft 11 which extends vertically upward to the exterior of the container and is driven by any suitable source of power. Rotation of the impeller is effective to agitate the contents of the container 1, drawing the liquid and suspended ore through the passage 10 and forcing them upward through the chamber 5 and causing them to circulate as indicated by the arrows.

As shown, surrounding the shaft 11 is a tube 13 placed in communication with the atmosphere above the surface of the liquid by a conduit 15, which latter may be provided with a valve 17. In operation the impeller 9 causes atmospheric air to be drawn through the conduit 15 and tube 13 and to discharge into the liquid for mixing with and aerating the same, the amount of air admitted being controlled by the valve 17.

The metal-value-bearing froth thus formed collects on the surface of the liquid, said sur-

face indicated at 19, and discharges from the container through a spout 20.

According to one form of the invention, the froth may be caused to pass between electrodes 21 and 23, the electrode 23 as shown being positioned adjacent the surface of the liquid and the electrode 21 being positioned above said surface. As illustrated, the two electrodes may be adjustably secured in selected positions longitudinally of a rod 25 of insulating material, say hard rubber, by means of set screws 27, said rod being carried by a bracket 29 secured to the walls of the container. As shown, to the upper electrode 21 is secured a wire 31 leading to one terminal of a suitable source of electromotive force, while the opposite electrode 23 is connected to the other terminal of said source by an insulated wire 33, which latter may be carried in the longitudinally extending slot 35 formed in the rod 25. Preferably a direct current source of electromotive force is employed, although beneficial results will be secured by employment of an alternating current source, particularly when the latter is of rather low frequency, say in the order of 25 cycles or less per second.

Preferably the electrodes are placed so that the rising oil bubbles from the chamber 5 as they reach the surface of the liquor are within the electrostatic field surrounding the electrodes. In the practice of the invention I have found that action of the electrodes 21 and 23 will increase the recovery of the ore. For example, in treating Southeast Missouri galena, which is essentially galena with traces of sphalerite, containing various impurities principally iron sulphide, and assaying about 5% lead, the total recovery of galena under favorable conditions is increased to about 77.6% of the entire lead present when the electrodes are charged, as against a total recovery of 58.8% of the entire lead present when the electrodes are not employed, or if employed are not charged.

It will be understood that the ore before treatment is first ground, for example, with the above mentioned ore ground sufficiently to pass it through a 75 mesh screen, while the treating liquor has added thereto known re-

agents to depress the substances which are to remain in the tailings. For example, with the above ore, when the galena is to be separated, in which case the sphalerite (ZnS) and iron sulphide (FeS) are to remain in the tailings, the liquor may have added thereto the following reagents for 1000 parts of ore:

|                                          | Parts |
|------------------------------------------|-------|
| Sodium carbonate                         | 2.20  |
| 10 Sodium cyanide                        | 0.09  |
| Zinc sulphate                            | 0.28  |
| Potassium xanthate                       | 0.045 |
| Thiocarbanilid                           | 0.035 |
| Pine oil (General Naval Stores No. 15 5) | 0.025 |

It will be understood that with the above reagents the oily substances in combination with agitation and aeration cause the production of a froth consisting essentially of oil bubbles to which adhere the particles of ore. The water content is not critical, but preferably in the above example about 18 parts of water are used for each part of ore.

Preferably the electrodes are of relatively large area or are otherwise formed to produce an extensively distributed field, for example, in a laboratory size flotation machine having a capacity of 1000 grams of ore and 9 liters of water satisfactory results will be produced with electrodes about 4 inches square positioned substantially as shown in the drawing, with a potential difference between the electrodes of about 220 volts direct current, and with the upper electrode touching the top surface of the froth and lower electrode about touching the surface of the liquor. It will be understood in this connection that the layer of froth in a machine of this size will be from about  $\frac{1}{2}$  to 4 inches thick depending upon the conditions of operation. Under these conditions in the above example the current flow between the electrodes will vary from 1.5 to 0.1 amperes.

It will be understood, as commonly practised in the art of ore separation by froth flotation, that by employing suitable known reagents selected mineral contents of an ore can be separated in a similar manner to that in which the galena is separated in the above example, and that the invention is applicable to various ores capable of being separated by froth flotation.

Applicant's explanation of the above phenomena is that when the lead sulphide, for example, is separated the particle P of this mineral, Fig. 3, adheres to the oil bubble B something after the manner indicated by said figure. The lead sulphide particle is positive relative to the oil bubble, but the oil bubble has an opposite and larger charge than the said particle, thus causing the combined particle and bubble to be negatively charged, with the result that by making the electrode 21 continuously positive by use of a direct current source of electromotive force,

or intermittently positive by use of an alternating source of electromotive force, and the electrode 23 continuously or intermittently negative, each bubble with its particle is drawn or impelled upward from the surface of the liquid to increase the concentration. Applicant however advances this theory merely as explanatory of the phenomena which occurs, actual tests demonstrating the fact that charging the electrodes as above indicated increases the amount of the concentrate. For example, treating 327 grams of the above mentioned ore, with the electrodes charged at a potential of 220 volts direct current as above described, 41.92 grams of lead sulphide concentrate were recovered, while with the same ore, with the electrodes not charged, but 28.2 grams of concentrate were recovered, in each case the concentrate recovered as saying exactly the same percentage of lead. With a charge on the electrodes the recovery of lead sulphide from the ore is therefore about 77.6% as compared to 58.8% with the electrodes uncharged. Apparently, electrical conductivity of the froth is necessary for the occurrence of the above phenomena, but so far as known to applicant all froths produced in flotation processes possess this property.

It will be understood that wide deviations may be made from the above described examples of method, apparatus and materials, without departing from the spirit of the invention.

I claim:

1. The process of ore separation which comprises subjecting an ore pulp to froth flotation to produce a metal-value-bearing froth over the froth liquor, and electrically attracting the metal-value-bearing fractions of said froth upward relative to the surface of said liquor by causing the froth to pass between electrodes having opposite electrical charges at a relatively high potential difference, one of which electrodes is above the surface of the liquor in electrical contact with the froth.

2. The process of selective sulphide ore separation which comprises subjecting an ore pulp to froth flotation to produce a sulphide-bearing froth over the pulp liquor, and electrically attracting the sulphide-bearing fractions of said froth upward relative to the surface of the liquor by causing the froth to pass between electrodes having opposite electrical charges at a relatively high potential difference, one of which electrodes is above the surface of the liquor in electrical contact with the froth.

3. The process of separating galena from ore containing other minerals which comprises subjecting an ore pulp to froth flotation to produce a galena bearing froth, and electrically attracting the galena-bearing fractions of said froth upward relative to

the surface of the liquor by causing the froth to pass between electrodes having opposite electrical charges at a relatively high potential difference, the electrode with a positive charge being above the surface of the liquor in electrical contact with the froth.

4. Apparatus for separating ores by froth flotation having, in combination, a container for ore pulp comprising a froth producing liquor, means for aerating said pulp to form on the pulp liquor a layer of metal-value-bearing froth, and a pair of opposed electrodes, one adjacent the surface of the liquor and the other carried above said surface in substantially insulated relation to the liquor.

5. Apparatus for separating ores by froth flotation having, in combination, a container for ore pulp comprising a froth producing liquor, means for aerating said pulp to form on the pulp liquor a layer of metal-value-bearing froth, and a pair of opposed plate-like electrodes of material area, one adjacent the surface of the liquor in substantially parallel relation thereto and the other carried above said surface in substantially insulated relation to the liquor.

6. Apparatus for separating ores by froth flotation having, in combination, means for agitating ore with a froth producing liquor to produce ore pulp, means for aerating said ore pulp to form on the pulp liquor a layer of metal-value-bearing froth, and a pair of opposed electrodes between which the froth is adapted to pass, one of said electrodes being adjacent the surface of the liquor and the other being carried above said surface in substantially insulated relation to the liquor.

7. Apparatus for separating ores by froth flotation having, in combination, means for agitating ore with a froth producing liquor to produce ore pulp, means for aerating said ore pulp to form on the pulp liquor a layer of metal-value-bearing froth, and a pair of opposed plate-like electrodes of material area between which the froth is adapted to pass, one of said electrodes being adjacent the surface of the liquor in substantially parallel relation thereto and the other being carried above said surface in substantially insulated relation to the liquor.

8. The process of ore separation which comprises subjecting an ore pulp to froth flotation to produce a metal-value-bearing froth over the pulp liquor, and impressing sufficient electrical charge on the froth to attract the metal-value-bearing fractions of the latter upward relative to the surface of the liquor.

9. The process of ore separation which comprises agitating ore with a froth producing liquor to produce ore pulp, aerating said pulp to produce a metal-value-bearing froth over said liquor, and impressing sufficient electrical charge on the froth to attract the

metal-value-bearing fractions of the latter upward relative to the surface of said liquor.

In testimony whereof, I have signed my name to this specification.

LOUIS J. O'MALLEY.

**CERTIFICATE OF CORRECTION.**

**Patent No. 1,891,776.**

**December 20, 1932.**

**LOUIS J. O'MALLEY.**

It is hereby certified that the Certificate of Correction issued February 7, 1933, was erroneously drawn as to the word "froth" and that this Certificate should have read as follows; page 2, line 104, claim 1, for "froth", second occurrence, read "pulp"; and that the said Certificate should be read with this correction therein that the same may conform to the record of the case in the Patent Office.

Signed and sealed this 28th day of February, A. D. 1933.

(Seal)

**M. J. Moore,  
Acting Commissioner of Patents.**